

May 7, 1957

S. CONVERSE

2,791,529

PROCESS FOR BONDING A PREFORMED NON-WOVEN  
BAT TO A WOVEN TEXTILE SHEET

Filed Sept. 17, 1954



INVENTOR:  
SHERMAN CONVERSE.

BY

Eaton + Bell

ATTORNEYS.

# United States Patent Office

2,791,529

Patented May 7, 1957

1

2,791,529

## PROCESS FOR BONDING A PREFORMED NON-WOVEN BAT TO A WOVEN TEXTILE SHEET

Sherman Converse, Graniteville, S. C., assignor to Graniteville Company, Graniteville, S. C., a corporation of South Carolina

Application September 17, 1954, Serial No. 456,738

4 Claims. (Cl. 154—137)

This invention relates to fabrics and methods of preparing the same and more particularly to a textile fabric composed of a woven fabric and a non-woven fabric or bat bound together and adapted for use in the manufacture of wearing apparel such as lining for garments of all sorts and all kinds, and could be used for bed garments, gloves, foot-wear and hats. This fabric can also be used for the making of bags, for packing and shipping of various kinds of bulk materials such as sugar, cement and desiccants. In this case the woven fabric would furnish the strength and the non-woven material combined therewith the necessary impermeability. Its excellent wet strength would give it a decided advantage over paper. It could also be used in any place requiring a fabric which would furnish a combination of strength, impermeability, compactness and resilience in a lighter weight, lower cost fabric than would be possible in the case of either a woven or non-woven fabric alone.

The invention also relates to and is concerned with a new and improved textile fabric, coated or uncoated, and which is provided with a base or other fabric of a textile material such as cheese cloth but which may be of any desirable fibre and weave, having secured thereto by impregnation, a non-woven bat which may be formed at the time and fed in conjunction with a sheet of cheese cloth or other suitable fabric, or a non-woven bat can be manufactured and formed into rolls, as well as the cheese cloth and then the two rolls can be combined by passing the same simultaneously through an impregnating and binder solution to permanently bind the two sheets together, which sheets are then subject to a squeezing operation to squeeze the binder therefrom and then the sheets—that is, the non-woven sheet of material and woven sheet of material would be dried and rolled into a suitable roll. If desired, the binder through which the two sheets are passed can have admixed therewith suitable metallic powder, such as aluminum, or, if desired, after the sheets have been bonded together and dried and wound into a roll, they can be passed through a second mechanism which will apply a metallic coating by means of a conventional knife-coating machine and then the coating will be dried to remove therefrom the volatile solvents, after which the coated cloth can be wound into a suitable roll.

The advantage of the combination of a woven and non-woven material bonded together is that the woven fabric furnishes the necessary strength for handling in the calendering and coating operations, where coating is employed, and the fibres making up the non-woven fabric fill up the holes between the yarns of the woven fabric, such as cheese cloth, thus preventing undue penetration of the metallic coating through the woven fabric.

This combined fabric of non-woven and woven sheets has more tear and tensile strength than a non-woven fabric of equivalent weight and is more compact in resilience than a woven fabric of equivalent weight.

It is, accordingly, one of the prime objects of the invention to provide a textile fabric of this nature having

2

a base of woven fabric or textile material of any desired fibre and weave and having thereon and bonded thereto a bat or web of unwoven material and which two materials when being bonded together may be also subjected to metallic powders and suitable binder agents to impregnate the unwoven material with a metallic powder, thus giving it greater insulating properties when used as coat linings or to make it more durable when used for other uses herein specified.

10 Other objects will be apparent and will become obvious as a description of the invention proceeds.

Briefly stated, the process by which the foregoing insulating textile material is produced comprises: (1) Feeding a non-woven bat and a woven piece of textile material through suitable apparatus and subjecting the two sheets of material to impregnation with a suitable binder dispersion or solution having dispersed therein, if desired, the desired metallic powder, (2) heating the impregnated fabric to drive off the diluent of the binder formulation thus binding the metallic powder in place, (3) calendering the thus coated fabric, if desired, to iron the base coat and thus produce a smooth surface for application to the various uses herein described, (4) applying a protective coating to the bonded fabric, if and when desired, the 25 protective coating comprising an organosol containing instead of metallic powder, one or more coloring pigments, (5) heating the coated fabrics to drive off the diluent from the organosol to fuse the resin and the plasticiser in the organosol and bind the pigment in place and then (6) embossing or otherwise treating the top 30 coat to produce any desired patterns.

The base or under fabric employed in accordance with the invention may be one of those which are commonly in use today, and include fabrics made of natural fibres such as cotton, wool, silk, linen and ramie, as well as fabric prepared from synthetic fibres of cellulosic origin such as rayon, cellulose acetate, or any of the regenerated celluloses. Fabrics made from true synthetic fibres may also be employed and such fibres may be vinyl chloride-acetate copolymers, polyvinylidene chloride, as well as any synthetic linear condensation super polymers, such as linear polyamides, of which nylon is typical. Also, polyester fibres such as Dacron and fibres of polymerized acrylo-nitrile such as Orlon and Acrilon, as well as co-polymer fibres of acrylo-nitrile and polyvinyl chloride such as Dynel; also, glass fibres and protein fibres such as Vicaro. Of course, the base fabric may be in any desired pattern or color, printed or woven, or it can be plain white or dyed in any desired color.

50 Organosols consist of an appropriate synthetic resin dispersed with a plasticiser in a thinner or diluent, along with a stabilizer and filler, if deemed desirable.

Any appropriate binder may be employed in forming the combination fabric and can be any one or more of 55 quite a variety of rubber, resin or other types of adhesives either in solution or dispersion form but preferably as a water dispersion. The preferred type of binder is a so-called nitrile rubber latex. Nitrile rubbers are copolymers of acrylonitrile and butadiene. Typical formulations are as follows:

1.4 pints nitrile rubber latex  
.50 ounce Nonic 118 (penetrant)

1 gallon volume

65 1.0 pint nitrile rubber latex  
6.0 ounces Exad (polyvinyl ether plasticizer)  
6.5 ounces aluminium powder  
.50 ounce Nonic 118

70 1 gallon volume

In the foregoing formulations, Nonic 118 is a product

marketed by Sharples Chemicals, Inc. comprising polyethylene glycol tertdodecyl thio ether.

Other types of latices which can be used as a binder are polyvinyl chloride, polyvinyl chloride—polyvinylidene chloride, polyvinyl acetate, or butadiene styrene, or a mixture of two or more of the same. If desired, aluminum powder or colored pigments may be applied along with these dispersions.

After the combination fabric is formed by impregnation with the binder and drying same, it may then be coated with an organosol formulation containing aluminum powder and if desired, with a second organosol containing aluminum or other metallic pigments.

As plasticisers in the organosols there may be employed any of the common natural plasticisers, such as abietic acid esters, or any of the common esters such as dimethyl phthalate, dibutyl phthalate, diethyl phthalate (2 ethyl hexyl), di-D-butoxy ethyl phthalate, dicapryl phthalate and various phthalates, various adipates, butyl stearate and related esters, dibutyl sebacate, diethyl sebacate, methyl glycolate and various phosphates.

As thinners or diluents the following may be employed: benzene, toluene, and xylene which represent a moderate choice of aromatic thinners, while aliphatic hydrocarbons such as petroleum ether or hexane may be used. Typical proprietary thinners and diluents are: "Apcothinner" (A nontoxic, V. M. & P. Naphtha solvent prepared by straight-run overhead distillation. Sp. gr. 0.763; A. P. I. gr. 44.6; flash point, 52° F., viscosity in centipoises, 0.667 at 60° F., and 0.512 at 100° F.), "Sovasol" #3, "Sovasol" #4 (A series of petroleum solvents manufactured in two grades. The first grade (Sovasols 1, 2, 3, 4, 5 and 6) are straight run naphthas of varying boiling ranges.), Hi-Flash Naphtha, V. M. & P. Naphtha (Varnish Maker's & Painter's Naphtha. A grade of naphtha used mainly as a thinner for paints and varnishes. Distillation range is usually between 195° and 330° F.), "Solvesso" Xylo, "Solvesso" 100 and "Solvesso" 150 (A line of aromatic solvents prepared synthetically from petroleum. Grades available include Solvesso Toluol, Solvesso xylol, and Solvesso 100 and 150. The flash point of Solvesso 150 is 145–150° F.). Ester diluents or thinners include methyl formate, ethyl acetate, n-butyl acetate, anil acetate, 2-ethylhexyl acetate, methylamyl acetate, 2-ethylbutyl acetate, Cellosolve acetate, isobutyl propionate and butyl lactate. Also there may be employed the various Cellosolves such as ethylene glycol monethyl ether, propylene glycol monoethyl ether, etc., as well as Carbitol and butyl Carbitol. Similarly, chlorinated hydrocarbons such as methylene chloride, chloroform, carbon tetrachloride, ethylene dichloride and chlorobenzene may be used. Ketones such as acetone, methyl ethyl ketone, diisobutyl ketone, methyl isobutyl ketone cyclohexanone and similar volatile ones find use as diluents in the composition. Certain volatile ethers such as di-ethyl ether, dioxane, or diisopropyl ether as well as certain alcohols such as isobutanol, 2-ethylhexyl alcohol, and cyclohexanol have some use as diluents and thinners for some resins. The classes of diluents and thinners may also be used in admixture with each other consistent with the principles set forth.

Included in the foregoing list, many of the ketones and esters have the dual function in the organosol of being dispersants as well as thinners and diluents.

The organosols also preferably contain stabilizers such as fused lead stearate, basic lead phosphite, stabilizer A-5, stabilizer C-2, stabilizer G-18 and Victor stabilizers 53 and 85 and various fillers such as calcium carbonate, Whiting, "Surfex" (A precipitated calcium carbonate of the surface-coated type. It is used as an extender pigment, partial vehicle replacement, and dispersing aid in paints. Also used as a filler in vinyl resins, and as an extender pigment in printing inks.), "Atomite" (Mechanically ground calcium carbonate substantially free from

particles larger than 15 microns in diameter. Use: as a filler for rubber, paint, paper, etc.), etc.

As stated hereinbefore, the metal powder is dispersed through this organosol to form the insulating coating. Preferably the metal powder is of pure aluminum of such particle size that 99% thereof pass through a 325 mesh screen. However, the invention is not limited to aluminum powder since other metallic powders such as powders of copper, silver, iron, steel, brass, bronze, Monel metal, zinc, or any alloy of two or more of the foregoing, may be employed in powder form. Naturally, consideration of economics will dictate the selection of the metal or alloy employed.

Among the pigments found suitable for a color coating are, "Mapico" iron brown No. 420, "Mapico" lemon yellow, "Mapico" black, "Mapico" brown No. 418, "Titanox" A-168 LO (A grade of titanium dioxide modified for reduction of after-yellowing of resins and vehicles of organic coatings. It is 97% titanium dioxide and has a specific gravity of 3.9.), chrome green, medium, fast violet, lampblack, oiled carbon black, basic silicate white lead, basic sulfate white lead, blue basic lead sulfate, basic lead carbonate, "Asbestine" 3X (Natural, pure-white, fibrous magnesium silicate, 99% of which passes through a 325-mesh screen.). Of course, some of the foregoing come under the category of "fillers" and may be employed as such in the organosol.

In the coating compositions, the organosol is prepared according to the following general formulation:

|                     | Pounds     |
|---------------------|------------|
| Resin               | 100 to 150 |
| Plasticizer         | 40 to 100  |
| Stabilizer          | 2 to 6     |
| Filler              | 0 to 150   |
| Thinner and diluent | 15 to 120  |

For the color coating a desired color pigment is ground with a plasticizer on a three-roll mill to form a color paste in the following proportions:

|             | Pounds   |
|-------------|----------|
| Pigment     | 20 to 70 |
| Plasticizer | 80 to 30 |

This color paste is then added to and thoroughly mixed with the organosol in the following proportions:

|             | Pounds   |
|-------------|----------|
| Organosol   | 80 to 90 |
| Color paste | 20 to 10 |

In carrying out the process, an organosol composition is first prepared having the following formulation:

|                                   |      |
|-----------------------------------|------|
| Vinylite resin VYNV.1             | 100  |
| Diethyl phthalate (plasticizer)   | 60   |
| Basic lead phosphite (stabilizer) | 2    |
| Calcium carbonate (filler)        | 15   |
| Xylo (Thinner and diluent)        | { 14 |
| Apco thinner                      | 30   |

The foregoing ingredients are ground in a pebble mill for approximately 12 hours.

In order to disclose a specific embodiment of the invention, reference is now had to the accompanying drawing in which Figure 1 shows, in more or less schematic flow sheet form, the apparatus employed in carrying out the present process, while Figure 2 shows a cross section of the finished composite coated fabric.

Employed in the formation of the reinforced fabric from a bat of non-woven fibres and a sheet of woven material, preferably cheese cloth, there is employed a Curlator manufactured by the Curlator Corporation, of Rochester, N. Y. This comprises a breaker 10 into which the fibres are dumped and it has a driven conveyor 11 which has a plurality of teeth thereon which elevate the fibres and in their descent a draft of air picks the fibres off of the toothed conveyor 11 and passes them beneath a screen conveyor 12 which is driven on suitable rollers 13 and 14.

## 5

A suction draft of air is caused to pass through the screen conveyor 12 by a suction pipe 12a to cause the fibres to adhere to the lower reach of the screen conveyor 12. The loose fibres are fed by the belt 12 to a licker-in 15 which conveys the fibres to a condenser 16 which has a suction draft of air on its interior which causes the fibres to be formed into a web on the periphery of the condenser 16. The web of fibres is removed by suitable strip-off means from the condenser 16 and this web of fibres is indicated at 17 as passing over a driven conveyor 18 which delivers the web of fibres to feed rolls 20 where the web of fibres is joined with the fabric such as cheese cloth 22 emanating from a roll 23 and the web of fibres 17 joined with the fabric 22 to form a composite fabric 29 which passes between the driven rollers 20 and 21.

The rollers 20 and 24 have mounted thereon a screen belt 25 and there are also provided in addition to roller 21 rollers 26, 27 and 28 which carry a screen belt 30 and the composite fabric 29 is passed between the rollers 20 and 21 and between the screen belts 25 and 30 and these screen belts 25 and 30 pass between immersion rolls 33 and 34 to immerse the composite fabric 29 in the heretofore described binder solution 37 disposed in a pan or vat 38. The combined and saturated fabric sheet 22 and the web of fibres 17 are immersed by the roller 34 and then the rollers 24 and 28 extract the surplus binder solution from the composite fabric 29 which surplus drains back into the vat 38 and then the combined product is passed over a plurality of drying cans 40, 41, 42, 43, 44 and 45 and over guide rollers 46, 47 and on to a take-up roll 48.

Now, in this condition the bat is complete unless it is desired to apply a coating to the same. As previously pointed out, the metallic particles or aluminum coating can be mixed in the binder solution 37 and applied to the woven fabric and the non-woven fabric sheets as they are passed through the binder solution 37.

However, if it should be desired to apply a suitable coating to the combined fabric after it has been wound onto the take-up roller 48, then the take-up roller 48 can be positioned in position shown in Figure 2 and passed over a roller 50 and beneath a feed tank container 51 containing a coating solution and/or a pigment solution if it is desired to apply a pigment coating to the combined fabric and the coating material is fed from the tank 51 onto the fabric and a coating knife 52 spreads the pigment coating or metallic coating, whichever the case may be, onto the combined fabric 29 composed of the non-woven web 17 and the woven fabric 22.

After this coating has been applied, the fabric 29 is led through a drying oven which preferably may have a first and second zone, the first zone being designated at 60 and the second zone being designated at 61.

In the case of an organosol or plastisol coating after the formation of the combined fabric, there may be provided the drying chambers 60 and 61 with a wall 63 therebetween, this wall having a suitable slot through which the fabric will pass. In the first half, or first zone 60, the temperature is approximately 290° F. In the second half, or portion 61, the temperature is preferably around 400° F. The cloth is in each zone about 35 seconds. In other words, 35 seconds is consumed by the cloth traveling through each of the heated chambers 60 and 61.

The high temperature in the second heated chamber 61 is to fuse the resin, that is, to melt the resin particles in the plasticiser to form a continuous film. It must be particularly pointed out that both base and top coats are fused in this operation and there is some inter-fusing between the two coating layers to form a stronger and more stable coated fabric. The coated cloth as it emerges from the dryer is rolled up as before onto a roll 67.

Figure 3 in the drawing shows the completed coated fabric. The base or under fabric, namely, the cheese cloth and the like, is indicated at 22 and the bat of fibres

## 6

is indicated at 17. The coating of same is applied as indicated at 72.

The colored top coat, if desired, may be applied as a plastisol, which is a dispersion of resin and pigment in plasticiser only, with no volatile liquid being present, or as a lacquer in which case the resin binder is actually dissolved in volatile solvents rather than being dispersed in volatile liquids which are non-solvents for the resin. The plasticiser, stabilizer, filler and pigment are added to the resin solution. The lacquer is knife coated as in the case of the organosol or plastisol, but the fusing operation is not necessary as a continuous film is caused by evaporation of the resin solvent.

In the drawings and specification there has been set forth a preferred embodiment of the invention and although specific terms are employed, they are used in a generic and descriptive sense only, and not for purposes of limitation, the scope of the invention being defined in the claims.

20 I claim:

1. A process for preparing a flexible, resilient insulating, composite fabric useful in the manufacture of wearing apparel and the like and composed of a preformed, non-woven sheet of textile fibers and a woven sheet of textile fibers, which comprises feeding the two sheets, in superposed, surface-contact relation, through a binding solution containing metallic powder of simultaneously impregnate both the non-woven and woven sheets therewith, pressing excess binder solution from the composite fabric, and then heating the composite fabric to drive off the volatile liquid from the binder solution, thus leaving the binder and the metallic powder thoroughly and uniformly dispersed through both sheets of the composite fabric thus to cause said sheets to adhere securely one to the other.

2. A process for preparing a flexible, resilient insulating, composite fabric useful in the manufacture of wearing apparel and the like and composed of a pre-formed, non-woven sheet of textile fibers and a woven sheet of textile fibers, which comprises feeding the two sheets, in superposed, surface-contact relation, through a binding solution containing metallic powder to simultaneously impregnate both the non-woven and woven sheets therewith, pressing excess binder solution from the composite fabric, heating the composite fabric to drive off the volatile liquid from the binder solution, thus leaving the binder and the metallic powder thoroughly and uniformly dispersed through both sheets of the composite fabric thus to cause said sheets to adhere securely one to the other, coating at least one surface of the composite fabric with an organosol containing coloring pigments, and then heating the thus coated fabric to drive off the volatile liquid from the organosol and fuse the resin and the plasticizer of the organosol into and throughout the two sheets of the composite fabric.

3. A process for preparing a flexible, resilient, insulating, composite fabric useful in the manufacture of wearing apparel and the like and composed of a pre-formed, non-woven sheet of textile fibers and a woven sheet of textile fibers, which comprises feeding the two sheets, in superposed, surface-contact relation, through a binding solution to simultaneously impregnate both the non-woven and woven sheets therewith, pressing excess binder solution from the composite fabric, heating the composite fabric to drive off the volatile liquid from the binder solution, thus leaving the binder thoroughly and uniformly dispersed through both sheets of the composite fabric thus to cause said sheets to adhere securely one to the other, coating at least one surface of the composite fabric with an organosol containing a metallic powder, and then heating the thus coated fabric to drive off the volatile liquid from the organosol and fuse the resin and plasticizer of the organosol into and throughout the two sheets of the composite fabric.

4. A process for preparing a flexible, resilient, in-

7

sulating, composite fabric useful in the manufacture of wearing apparel and the like and composed of a pre-formed, non-woven sheet of textile fibers and a woven sheet of textile fibers, which comprises feeding the two sheets, in superposed, surface-contact relation, through a binding solution to simultaneously impregnate both the non-woven and woven sheets therewith, pressing excess binder solution from the composite fabric, heating the composite fabric to drive off the volatile liquid from the binder solution, thus leaving the binder thoroughly and uniformly dispersed through both sheets of the composite fabric thus to cause said sheets to adhere securely one to the other, coating at least one surface of the composite fabric with an organosol containing metallic powder, heating the thus coated fabric to drive off 15 the volatile liquid from the organosol, superposing on

5

said first organosol coating another organosol coating containing coloring pigments, and then heating the thus coated fabric to drive off the volatile liquid from the second organosol and fuse the resins and plasticizers of both organosols into and throughout the two sheets of the composite fabric.

8

## References Cited in the file of this patent

## UNITED STATES PATENTS

|    |            |                 |               |
|----|------------|-----------------|---------------|
| 10 | Re. 23,741 | Summers         | Nov. 17, 1953 |
|    | 1,408,871  | Enos            | Mar. 7, 1922  |
|    | 2,125,341  | Hall et al.     | Aug. 2, 1938  |
|    | 2,275,989  | Perry           | Mar. 10, 1942 |
|    | 2,528,168  | Paulsen         | Oct. 31, 1950 |
|    | 2,706,699  | Plansoen et al. | Apr. 19, 1955 |